

# UNITED STATES PATENT OFFICE.

WILLIAM G. ROACH, OF CINCINNATI, OHIO, AND ALBERT C. ROACH, OF NEWPORT, KENTUCKY, ASSIGNEES, BY MESNE ASSIGNMENTS, TO THE CINCINNATI CHROME LEATHER COMPANY, OF CINCINNATI, OHIO, A CORPORATION OF OHIO.

## PROCESS OF TANNING HIDES, SKINS, AND THE LIKE.

No. 839,904.

Specification of Letters Patent.

Patented Dec. 25, 1906.

Application filed March 4, 1904. Serial No. 196,587.

*To all whom it may concern:*

Be it known that we, WILLIAM G. ROACH, residing at Cincinnati, in the county of Hamilton and State of Ohio, and ALBERT C. ROACH, residing at Newport, in the county of Campbell and State of Kentucky, citizens of the United States, have invented certain new and useful Improvements in the Process of Tanning Hides, Skins, and the Like, of which

10 the following is a specification.

The object of our invention is to provide a process for the metallic tanning or tawing of hides which produces a leather having substantially the same capacity for finishing, 15 working, or use as bark-tanned leather while retaining the toughness and durability of the metallic-tanned leather.

It consists, broadly speaking, in introducing into the fibers of the hides in a substantially inactive chemical state substances, 20 containing tanning matter adapted to be released by reaction between said compounds and then establishing a condition under which said reaction will take place. We 25 prefer to employ chromic acid as the substance containing the tanning matter and introduce it into the hide in substantially the same form and manner as in the first bath of the ordinary "two-bath" process. After 30 the hide has become thoroughly soaked and impregnated with the chromic acid we introduce a reducing agent, such as glucose, which does not act at once upon the chromic acid, but is what may be termed "chemically inactive" for the time being toward 35 said acid. When the hide has become thoroughly soaked and impregnated with the glucose, it will be seen that the chromic acid and glucose are intimately and uniformly associated together and with the fibers of the hide.

40 Thus, in effect, we bring each molecule of the chromic acid into intimate association with its molecule of glucose on the particular fiber upon which their product is to act before 45 said product is released. Under these circumstances when the reaction does take place the chromic acid is deposited directly and immediately upon the hide fibers. As 50 the chromic acid and glucose are uniformly distributed throughout the hide fiber, it will be seen that the chromic acid will also be uni-

formly deposited thereon and the interior fibers will receive their due proportion of the oxid.

In practice for one hundred pounds of 55 hides we employ as the first bath six pounds of bichromate of potash or soda, four pounds of alum, four to six pounds of common salt, twelve ounces of sulfuric acid, twenty ounces of hydrochloric acid, sixty gallons of water. 60 The hides to be treated are prepared in the usual manner for tanning and allowed to soak in this bath until thoroughly impregnated with the chromic acid. This will ordinarily take from twelve to eighteen hours, 65 depending upon the weight and thickness of the hides. The hides are then removed from the bath, "slied," "set out," and hung up until about three-fourths of the moisture therein has evaporated. When in this state, 70 the hides are spread out and painted on both sides with a solution of glucose and packed in piles for from three to six hours to allow the glucose to soak in and become uniformly distributed throughout the hide. The glucose 75 solution may contain from fifteen to fifty per cent. of glucose dissolved in water. If applied under ordinary atmospheric temperatures, there will be substantially no immediate reaction between the glucose and 80 chromic acid, they being under the conditions applied in an inactive state toward each other. Thus the glucose will soak into the hide and thoroughly and uniformly associate 85 itself with the chromic acid and hide fibers before any reducing action takes place. By painting the glucose solution onto the hide possible contact between the chromic acid in the hide and the glucose solution from which the painting-supply is taken is prevented. 90

To prevent the glucose from souring in warm weather, we use for, say, three gallons of water, about a half-pound of quassia chips, and, say, a half an ounce of carbolic acid. The quassia chips are boiled with the water 95 and the carbolic acid added, and into this is stirred the glucose to make up the necessary strength of the solution.

In the chromic-acid bath a small excess of 100 sulfuric and hydrochloric acid tends to hasten the reduction. If a larger excess of acid be used, the reduction will take place in a pro-

- portionately shorter time. Thus if it is desired to hasten the reduction an excess of acid, preferably sulfuric acid, may be employed; but care should be taken that the excess of acid is not enough to cause the reduction before the glucose is uniformly distributed through the hide or cause the acid to injuriously affect the hide fiber. We prefer to use glucose as the reducing agent.
10. All organic substances have more or less reducing action on chromic acid, and we think that an organic compound will generally be found preferable to employ as a reducing agent, since their action is generally slower. However, even an inorganic reducing agent may be employed if the proper conditions are obtained for preventing immediate reduction. After the hides have been uniformly impregnated with the chromic acid and glucose a condition is established under which the reaction between said substances takes place to release the chromic acid or tanning substance. This condition may be established in a number of ways; but 15 we prefer to use a bath of hot grease for this purpose. After the hides have been treated with the glucose solution and about one-fourth of the moisture has evaporated therefrom they are immersed in a bath of hot grease, the proportions of the ingredients of this bath being dependent upon the purposes for which the leather is to be used.
- For the production of a suitable sole-leather we make up a bath as follows: one 20 hundred pounds stearic acid, twelve and one-half pounds carnauba-wax, six and one-fourth pounds vaseline, six and one-fourth pounds beeswax. This grease-bath is reduced to a liquid and kept at a temperature between 85° and 90° centigrade, and the hides are suspended in this bath until the 25 grease has thoroughly penetrated the thickest parts of the hide. This will be found to take only a comparatively short time, an hour or more being all that is necessary. The effect of the hot grease is to establish a condition under which the chromic acid is thoroughly reduced and at the same time the hide is thoroughly filled with grease. For 30 sole-leather the hides are then rolled and finished in the usual way. For harness-leather the proportion of vaseline in the stuffing-bath must be increased to make the leather as soft as wanted—say twenty-five pounds of vaseline instead of six and a quarter pounds, as above stated. To obtain the best results, the glucose should be kept at about 50° centigrade.
- While our process attains its greatest utility in tanning thick or heavy hides, it may also be used to advantage for thin hides and will be found to produce a high grade of uniformly-tanned leather.
- 60 We claim as our invention—
- 65 1. The process of tanning hides which con-

sists in introducing into the fibers of the hide, in a substantially inactive chemical state, substances containing tanning matter adapted to be released by reaction between said substances, and then establishing a condition under which said reaction will take place, substantially as specified.

2. The process of tanning hides which consists in introducing into the fibers of the hide, in a substantially inactive chemical state, substances containing tanning matter adapted to be released by reaction between said substances, and then applying heat to establish a condition under which said reaction will take place, substantially as specified.

3. The process of tanning hides which consists in introducing into the fibers of the hide, in a substantially inactive chemical state, substances containing tanning matter adapted to be released by reaction between said substances, and then subjecting the hide to a bath of hot grease to establish a condition under which said reaction will take place, substantially as specified.

4. The process of tanning hides which consists in introducing a reducible metallic substance into the fiber of the hide; then introducing a reducing agent into the hide fiber in a substantially inactive chemical state toward said metallic substance; and then establishing a condition under which reduction will take place, substantially as specified.

5. The process of tanning hides which consists in introducing a reducible metallic substance into the fiber of the hide; then introducing a reducing agent into the hide fiber in a substantially inactive chemical state toward said metallic substance; and then applying heat to establish a condition under which reduction will take place, substantially as specified.

6. The process of tanning hides which consists in introducing a reducible metallic substance into the fiber of the hide; then introducing a reducing agent into the hide fiber in a substantially inactive chemical state toward said metallic substance; and then subjecting the hides to a bath of hot grease to establish a condition under which reduction will take place, substantially as specified.

7. The process of tanning hides which consists in subjecting them to a bath of chromic acid; then to that of an organic reducing agent, substantially inactive chemically toward the chromic acid; and then establishing a condition under which reduction will take place, substantially as specified.

8. The process of tanning hides which consists in subjecting them to a bath of chromic acid; then to that of an organic reducing agent, substantially inactive chemically toward the chromic acid; and then to a bath of hot grease to cause the reduction, substantially as specified.

9. The process of tanning hides which con-

sists in subjecting them to a bath of chromic acid; then to that of a solution of glucose under conditions in which the chromic acid and glucose are chemically inactive; and then establishing a condition under which the chromic acid is reduced by the glucose, substantially as specified.

10. The process of tanning hides which consists in subjecting them to a bath of chromic acid, then painting the hides with a reducing agent chemically inactive toward the chromic acid, and then establishing a condition under

which reduction will take place, substantially as specified.

11. The process of tanning hides which consists in subjecting them to a bath of chromic acid, then painting the hides with a solution of glucose, and then subjecting them to a bath of hot grease, substantially as specified.

WILLIAM G. ROACH.  
ALBERT C. ROACH.

Witnesses:

GLENA PRITCHARD,  
O. M. ROGERS.